

(No Model.)

W. E. INGLIS.

PROCESS OF AND APPARATUS FOR EXTRACTING METALS FROM ORES.

No. 596,458.

Patented Dec. 28, 1897.

*Fig. 1.*



*Fig. 3.*



*Fig. 2.*



WITNESSES:

L. N. Legendre  
M. A. Boyle

INVENTOR

Walter E. Inglis  
BY  
Thomas Drew Wilson  
ATTORNEY

# UNITED STATES PATENT OFFICE.

WALTER E. INGLIS, OF MOUNT VERNON, NEW YORK.

## PROCESS OF AND APPARATUS FOR EXTRACTING METALS FROM ORES.

SPECIFICATION forming part of Letters Patent No. 596,458, dated December 28, 1897.

Application filed April 20, 1896. Serial No. 588,291. (No model.)

*To all whom it may concern:*

Be it known that I, WALTER E. INGLIS, residing at Mount Vernon, in the county of Westchester and State of New York, have invented certain new and useful Improvements in the Process of and Apparatus for Extraction of Metals from Ores by the Use of Electricity; and I do hereby declare the following to be a full, clear, and exact description of the process and apparatus, such as will enable others skilled in the art to which it appertains to make use of the same.

This invention relates to the recovery or separation of metals, precious or other, from their ores, its application not being confined to any particular ore or metal. In the following specification I have described it as applied to the extraction of tin from its ores.

I take a crucible made of a suitable non-electroconducting material and first place therein a quantity of metallic tin sufficient when melted to cover the bottom of the crucible. This mass of molten metal is connected to the negative pole of a dynamo or other convenient source of electricity by means of a wire or other suitable conductor and forms the cathode of the electrolytic bath wherein the ore is to be treated. I next place in the crucible a sufficient quantity of chlorid of sodium or other substance capable of being decomposed by the electric current and containing a more electropositive element than the metal in the ore to be treated. This forms the electrolyte and is kept in a molten state at a temperature above the volatile point of metallic sodium at first by means of outside heat, but afterward the electric current is passed through it in such quantity that enough heat is developed in its passage to keep the whole bath at the proper temperature. In this bath and on top of the molten cathode and in direct contact with it is placed a quantity of properly crushed and concentrated tin ore, the metal of which it is purposed to extract. The anodes of the electric bath consist of one or more carbon rods which reach down into the crucible and are immersed for part of their length in the electrolyte of fused salt. These anodes are supported in any convenient manner and are connected by a conductor to the positive pole of the dynamo or other source of electricity. A continuous current of elec-

tricity at about five volts and of sufficient quantity to maintain fusion is passed through the bath. This decomposes the electrolyte, separating it into its elements, chlorin and sodium, the chlorin passing from the bath at the carbon anodes and either escapes into the atmosphere or is conducted into a flue and disposed of as it may be convenient. The sodium, being the electropositive element of the electrolyte, passes to the cathode at the bottom of the bath, and as the temperature is above the volatile point of sodium is volatilized, and having more affinity for the oxygen which is in combination with the tin in the ore unites with it, forming oxid of sodium, and displacing the tin sets it free in a molten state. The tin thus separated from the oxygen sinks into and increases the layer of melted tin below.

In order to utilize in the reduction of ore all the sodium produced by the electric current and also to prevent the sodium from alloying itself with the metal produced, I allow the metal after reduction to percolate in a finely-divided molten condition at a temperature above the volatile point of sodium through ore which has not been acted on. This is accomplished by raising the molten surface of metal which serves as the cathode above the bottom of the crucible. This leaves a groove all around the raised portion, ending in the tap-hole. This groove contains ore not yet acted on, and the metal in the elevated cathode being constantly increased by addition of reduced metal overflows and percolates through the interstices of the ore. By this method any sodium which may have alloyed itself with the reduced metal is by reason of the high temperature, assisted by the finely-divided state of the metal, rendered volatile and reduces the fresh ore which is in contact with it. Another reason for raising the cathode above the main body of reduced metal is that any slag that may be formed during the operation, consisting of silicates heavier than the electrolyte and which by their gathering around the cathode would interfere with the proper operation of the bath and tend to contaminate it, will fall away from the cathode and remain in the groove around it above the reduced metal and, as the metal is tapped, will follow it out of the crucible and be dis-

posed of as most convenient. As the operation continues the bath is gradually changed from chlorid of sodium to oxid of sodium, which under the action of the electric current 5 is resolved into oxygen and sodium, the oxygen being liberated at the carbon anodes and the sodium, as before, being substituted for the metal at the cathode and converted into oxid of sodium, which is continually produced 10 as fast as it decomposes, leaving the metal of the ore in a metallic state.

The following is a description of the best means of carrying out the invention and for the utilization of all the reducing agents produced by the electric current. 15

The drawings herewith form part of this specification.

Figure 1 is a central vertical section. Fig. 2 is a plan view; and Fig. 3 is a section corresponding to Fig. 1, but showing a modification. 20

In all the figures similar letters of reference indicate corresponding parts of the apparatus.

I provide a furnace of fire-brick or other 25 suitable material provided with a gas-burner or other conveniently-used source of heat, which, however, is mainly essential at the commencement of the operation, the current being of such quantity that the heat developed 30 by the resistance of the bath is sufficient to keep it in a state of fusion.

Within the furnace I mount a crucible A, having at the bottom an elevated central portion A', the top of which is hollowed to constitute 35 a basin *a*, preferably of circular form, adapted to receive and retain a melted mass of metal which presents an extended surface. The rim A' around this central pool should be as nearly level as possible, so that the 40 overflow may extend over a large portion of the surface as the melted metal accumulating in the basin *a* overflows to gather in the circular groove *a'* below. I provide for tapping out the metal from this groove through a tap 45 *a'*, formed in the extension, as shown in Fig. 1.

B' is a support, of iron or other suitable conducting material, extending across the top of the crucible and carrying a number of carbons B, which may be shifted downward in 50 the support from time to time as consumed. These connect through the support and by means of a wire B<sup>2</sup> with the positive pole of a dynamo M, which may be at any convenient distance and driven by a steam-engine or 55 other power, so as to afford a proper current of electricity.

I supply a sufficient quantity of chlorid of sodium (common salt) to make, when fused, a bath which shall occupy all the otherwise 60 unfilled space in the lower portion of the interior of the crucible. This serves as the electrolyte.

D is a hollow shield, which may be of the same material as the crucible, open at the 65 top and bottom and extending above the surface of the electrolyte. The lower end of this shield is flared, as indicated by D'. Through

this shield I introduce the broken ore G either constantly or at short intervals, so as to maintain it nearly or quite filled. This shield keeps 70 the volatile sodium separate from the general mass of the electrolyte and confines it to the unreduced body of ore within the shield. This construction also prevents the ore from ever being received in the general body of 75 the crucible in such quantity as to come in contact with the carbons.

A quantity of tin, sufficient when melted to fill the cup-like cavity or basin *a*, is introduced therein and when the apparatus is in 80 operation forms a circular extended surface of highly-conducting material which serves as the cathode. A conductor E, of metallic wire, or it may be of other material, extends upward from this melted tin through a non-conducting sheath F, which may be of the same material as the crucible or of any other suitable material, and connects to the negative pole of the dynamo. When the apparatus is in operation, there is a constant flow 85 of the current from the carbon down through the electrolyte to the cathode and thence upward through the conductor back to the dynamo.

Tin ore G, properly crushed and concentrated, being supplied through the liberal space within the shield my apparatus maintains 95 a covering of ore not only over the cathode, but also over the whole bottom of the interior of the crucible. 100

A current at five volts serves to decompose the electrolyte, the chlorin passing from the bath at the anode and the sodium going to the cathode, there substituting itself for the oxygen of the ore, as already described. By 105 this reaction oxid of sodium is produced, which remains in the bath, the quantity of which constantly increases until the whole bath is changed to fused oxid of sodium, which, like the chlorid, is decomposed, the sodium as before acting on the ore and the oxygen passing from the bath at the anode. As oxid of sodium unites with stannic oxid to form fusible sodium stannate, this salt may be formed as an intermediate product, 115 but as it is easily decomposed under the action of the electric current into its elements—sodium, tin, and oxygen—it will result finally as described, the tin and sodium going to the cathode and the oxygen passing from the bath 120 at the anode. Thus it will be seen that I provide a continuous process of separating metals from the elements associated with them in their ores, the associated element first passing from the ore to the electrolyte under the 125 reducing action of an element of a superior electropositive affinity derived from the electrodecomposition of the electrolyte itself and finally passing from the bath at the anode under the action of the electric current. The 130 tin after its separation sinks into the molten surface of the cathode, causing it to overflow and pass in a finely-divided condition at the temperature of the bath through ore not as

yet acted upon, as already explained. This will prevent any sodium remaining alloyed with the reduced metal. Any silicious material in the ore not capable of reduction will be converted into fusible silicates and being heavier than the electrolyte will fall away from the cathode and lie on top of the reduced metal and will be tapped off after it.

When the ore to be operated on is itself a tolerably good conductor of electricity, it can serve as the cathode, even without the layer of reduced metal being in contact therewith, by simply having the conductor F come in contact with the heated ore for a sufficient distance, as shown in Fig. 3; but for ores of ordinary conductivity I prefer to work with the reduced metal and the ore, both together to serve as the cathode.

I claim as my invention—

- 20 1. The within-described method of extracting metals from ores or compounds, consisting in electrically decomposing an electrolyte, comprising an agent of more electro-positive character than that of the metal in the ore, or compound and causing the freed agent to displace the metal in the ore or compound, and afterward passing the reduced metal at a high temperature in contact with a body of untreated ore or compound to free 25 it from residual traces of said agent; all substantially as, and for the purpose set forth.
- 20 2. An apparatus for electrically extracting metals, consisting of the combination of a crucible adapted to contain metallic compounds, an electrolyte, and refractory anodes B, means for retaining in the interior of the crucible, an extended surface of melted metal,

elevated above the main portion of the bottom and forming the cathode, the rim A<sup>2</sup> being adapted to distribute the overflow so as 40 to present to further unreduced ore, an extended surface of melted metal as it descends, and a receptacle for receiving the melted overflowings from the rim A<sup>2</sup>, and provided with a plug substantially as, and for the purpose set forth. 45

3. In apparatus for reducing metals by aid of electricity, the combination of a crucible and inclosing furnace, provisions for generating heat at the commencement of the operation, provisions for tapping out the reduced metals and for supplying more material, and a source of electricity, conductors therefrom, and electrodes B connected to serve as the anode, an elevated pool of melted metal a to 55 act as the cathode, a wire E therefor, with its inclosing sheath F and a further inclosing cylinder D, having a flared lower flange D' all combined and arranged as set forth.

4. The process of extracting tin from a refractory ore, consisting in liberating from a fused sodium compound, by the action of an electric current, the sodium, and causing the freed nascent sodium to separate the tin without fusing said tin and finally collecting 60 65 the tin.

In testimony that I claim the invention above set forth I affix my signature in presence of two witnesses.

WALTER E. INGLIS.

Witnesses:

J. B. CLAUTICE,  
M. F. BOYLE.